

Dec. 16, 1969

P. Y. KARINTHI ET AL  
METHOD OF IMPROVING THE PROPERTIES OF A FERROUS  
METAL IN THE MOLTEN STATE  
Filed Sept. 26, 1966

3,484,232



**Fig.2**



**Fig.3**



INVENTOR

PIERRE YVES KARINTHI  
ETIENNE SPIRE  
By Young & Thompson  
ATTYS.

3,484,232  
METHOD OF IMPROVING THE PROPERTIES OF A FERROUS METAL IN THE MOLTEN STATE  
Pierre Yves Karinthi, Champigny-sur-Marne, France, and Etienne Spire, Montreal, Quebec, Canada, assignors to L'Air Liquide, Societe Anonyme pour l'Etude et l'Exploitation des Procedes Georges Claude, Paris, France

Filed Sept. 26, 1966, Ser. No. 581,920

Claims priority, application France, Oct. 21, 1965, 35,745; Aug. 10, 1966, 72,625

Int. Cl. C21c 7/00

U.S. Cl. 75—45

12 Claims

## ABSTRACT OF THE DISCLOSURE

A halogenated compound is brought in liquid phase into contact with a porous device which on its opposite side contacts molten ferrous metal. The halogenated liquid is forced by gas pressure through the porous device and into the molten metal. The halogen may be used to remove unwanted elements from the metal. The non-halogen part of the compound may combine with elements dissolved in the metal or may itself dissolve in the metal.

This invention relates to a method of improving the properties of a steel or a cast iron by treating it in the molten condition.

The invention is characterised by the fact that there is injected into the molten metal, in the liquid or vapour state, mixed or not mixed with inert gas, through a permeable wall, a halogenated compound which is forced through said wall by gas pressure and which, having possibly decomposed on contact with the molten metal or in contact with a sufficiently hot portion of permeable wall, reacts chemically with the molten metal and improves the properties of the metal obtained, either by modifying its quality, or by modifying its composition.

This injection enables use to be made of halogens, or elements combined therewith, or both in a form easy to handle and often less onerous than when these reagents are used as in the prior art. In addition, the method of injection, which is easy to carry out, imparts great efficiency to the reagents because they are thereby finely distributed in the liquid metal.

The following uses of the method of the invention, which are merely non-limitative examples can be quoted:

(A) Selective elimination and possibly recovery of the manganese in cast iron intended in particular for the manufacture of cast iron comprising spheroidal graphite in a ferritic matrix, for example, by means of carbon tetrachloride, trichlorethylene, perchlorethylene, poly-halogenated derivatives of the hydrocarbons marketed under the name "Freons," and lead dichloride. These reagents react through their halogens which combine with the manganese to give a volatile compound.

By way of example, a 100 kg. charge of a cast iron containing:

|    | Percent |
|----|---------|
| C  | 3.8     |
| Si | 0.8     |
| Mn | 0.85    |
| P  | 0.1     |

was treated by blowing in liquid  $CCl_4$ .

After blowing in 2.2 kg. of  $CCl_4$  for six minutes, the manganese content was brought to 0.06%, the silicon content remaining unchanged. Thus, 93% of the initial manganese was eliminated.

(B) Fixing the carbon, for example by means of titanium trichloride, titanium tetrachloride, zirconium tetrachloride and niobium pentachloride, particularly in stain-

less steels, extra-mild steels for sheet intended for enameling, and in all ferrous metals in which this fixation is beneficial. These reagents react through their metal. It is known that certain ferro-titaniums, notably the conventional composition containing 30% of titanium, are difficult to dissolve in ferrous metals.

(C) Incorporation of small quantities of an element to give increased efficiency, for example the addition of boron to steels by the introduction of boron trichloride.

(D) Refining the grain of steel, for example by the introduction accompanied by increased yield, of niobium pentachloride in carbon steels for sheets having a high elastic limit and intended, for example, for use in the manufacture of pipes for carrying fluids under pressure; the niobium resulting from the decomposition of its chloride refines the grain of the steel.

The above-mentioned elimination of manganese is achieved by halogenation using inexpensive reagents and the method of introduction used gives a high yield on the part of the reagent because it is thereby finely distributed in the liquid metal. Furthermore, the recovery, from the fumes given off, of the manganese chloride, provides a valuable by-product. This elimination generally calls for 1.3 to 5 kg. of chlorine per kg. of manganese to be removed: carbon tetrachloride, if this is used for the injection, contains 92% of chlorine. The recovery of the manganese can be carried out by bringing the vapour into contact with water which dissolves the manganese chloride and iron chloride, the iron chloride being precipitated, then by subjecting the remaining solution to electrolysis, to obtain the manganese.

The incorporation of small quantities of an alloying element, using a compound which decomposes, has already been proposed. The compound in question was a metal carbonyl which is a costly reagent; furthermore, it would have been poorly utilised because it was proposed to introduce it through a single orifice which would have produced large bubbles. The present invention, on the other hand, permits the use of a relatively inexpensive reagent, and permits it to be employed very efficiently, in contrast to the conventional ferro-alloys, the yields from which are in the order of 60%.

Generally, the weight of reagent introduced does not exceed 1% of the weight of the metal treated.

The invention will again be described hereunder by reference to the attached drawing in which:

FIGURE 1 represents the general arrangement of the treatment vessel and of the auxiliary vessel for introducing the reagent;

FIGURE 2 shows a different embodiment of the same general arrangement;

FIGURE 3 represents a variant in which the auxiliary vessel is in the form of a plunger tube having a permeable base;

FIGURE 4 shows a variant of the equipment of FIGURE 2, in which the reagent is vaporized before being introduced.

In FIGURE 1 there is shown a vessel 1, the base of which is provided with a permeable plug 2. The rear portion of this plug is surrounded by a fluid-tight envelope 3 connected by a pipe 4 to an auxiliary vessel 5 containing the halogenated compound to be forced into the plug. The pipe 4 passes into this vessel through a plunger tube 6. A pipe 7 connects the vessel 5 to a gas cylinder 8, provided with a control valve 9 and a manometer-flowmeter unit 10. The vessel 5 is further provided with a discharge pipe 11 fitted with a valve 12. Finally, the vessel 5 can be placed on a balance 13 so as to facilitate the measuring out of the liquid forced via the pipe 4 and control valve 14 through the porous plug.

FIGURE 2 represents a variant in which the auxiliary

vessel 34 is attached to the treatment vessel 1 and is fixed in a fluid-tight manner beneath the base of this latter vessel.

A forcer pipe is arranged in the form of a plunger tube 37 directed towards the base of the auxiliary vessel. As previously, this latter vessel is provided with a pressurizing pipe 7 connected to a gas cylinder 8, and with a discharge pipe 11. Finally, it is optionally provided with heating means represented symbolically by an electric coil 15. This could be a resistance or an inductance coil, or could even be replaced by a spiral steam pipe.

The halogenated compound can thus be loaded into the auxiliary vessel in the solid condition, then melts when it is to be forced up through the porous plug 2.

If need be, the halogenated compound could initially be contained, in the solid, liquid, or even gaseous state, in an ampoule or a sealed cartridge fitted with a fusible plug or with a plug which could be broken by a magnetic hammer or any other equivalent means.

Optionally, treatment vessel 1 is provided with a fluid-tight cover 16 connected by piping 17 to a vacuum pump (not shown).

The injection equipment shown in FIGURE 3 is in the form of a refractory plunger tube 18 closed by a porous plug 19. The tube 18 has in its axis a cavity 20 surrounded by a coil 21 intended to melt the halogenated compound 22 previously introduced in the solid condition into the cavity 20. This cavity is connected by a pipe 23 to a source of inert gas, not illustrated.

The tube 18 is plunged into the bath of metal to be treated, in such manner that its porous mouthpiece 19 is located below the surface 24 of the bath.

FIGURE 4 shows a variation of equipment of FIGURE 2 in which the auxiliary vessel 34 is provided, at its base, with a porous plug fitted with a fluid-tight envelope 26 connected to a gas pipe 7. This vessel is optionally provided with a heating coil 15. The bubbling of gas through the plug 25 and then through the halogenated reagent brought to the region of its boiling point entrains a certain quantity of this reagent in the diluted vapour state. This diluted vapour, together with the gas enters the metal bath through the permeable element 2 which separates the treatment vessel 1 and the auxiliary vessel 34. In this manner, the reagent passes into the metal to be treated, forcing through a fluid-permeable wall pressure at the temperature obtaining in the auxiliary vessel.

What we claim is:

1. A method for improving the properties of a ferrous metal, comprising establishing a bath of molten ferrous metal to be treated, forcing through a fluid-permeable wall and into the bath a halogen-containing fluid that is chemically reactive with at least one component of the bath, the halogen of said fluid being present in the form of a halogenated compound selected from the class consisting of halogenated hydrocarbons and lead dichloride, said bath containing manganese to be at least partially eliminated by said halogenated compound, and recovering manganese from fumes evolved from the bath. 50

2. A method for improving the properties of a ferrous metal, comprising establishing a bath of molten ferrous metal to be treated, and forcing through a fluid-permeable wall and into the bath a halogen-containing fluid that is chemically reactive with at least one component of the bath, said halogen of said fluid being present in the form 60

of a halogenated compound selected from the class consisting of titanium trichloride, titanium tetrachloride, zirconium trichloride, and niobium pentachloride, said bath containing carbon to be fixed by said halogenated compound.

5 3. In a method for improving the properties of a ferrous metal, comprising establishing a bath of molten ferrous metal to be treated, and forcing through a fluid-permeable wall and into the bath a halogen-containing fluid that is chemically reactive with at least one component of the bath; the improvement comprising bringing said halogen-containing fluid into contact with said fluid-permeable wall as a liquid under pressure.

10 4. A method as claimed in claim 3, and applying pressure to said liquid by means of a gas under pressure.

5 5. A method as claimed in claim 3, the halogen of said fluid being present in the form of a halogenated compound the nonhalogen part of which remains in the bath.

15 6. A method as claimed in claim 5, said nonhalogen part being boron.

7. A method as claimed in claim 3, the ferrous metal being carbon steel and the halogen of said fluid being present in the form of a halogenated compound the nonhalogen part of which refines the grain of the steel.

25 8. A method as claimed in claim 3, the halogen of said fluid being present in the form of a halogen compound whose decomposition temperature is lower than the temperature of the bath.

9. A method as claimed in claim 3, the halogen of said fluid being present in the form of a compound whose decomposition temperature is lower than the temperature of at least a portion of said wall.

30 10. A method as claimed in claim 3, the halogen of said fluid being present in the form of a halogenated compound selected from the class consisting of halogenated hydrocarbons and lead dichloride, said bath containing manganese to be at least partially eliminated by said halogenated compound.

40 11. A method as claimed in claim 10, and recovering manganese from fumes evolved from the bath.

12. A method as claimed in claim 3, in which the halogen of said fluid is present in the form of a halogenated compound selected from the class consisting of titanium trichloride, titanium tetrachloride, zirconium trichloride, and niobium pentachloride, said bath containing carbon to be fixed by said halogenated compound.

#### References Cited

##### UNITED STATES PATENTS

|           |         |          |       |         |
|-----------|---------|----------|-------|---------|
| 2,134,905 | 11/1938 | Bamfylde | ----- | 75-59 X |
| 2,871,008 | 1/1959  | Spire    | ----- | 266-39  |

##### FOREIGN PATENTS

|           |         |                |
|-----------|---------|----------------|
| 590,537   | 1/1960  | Canada.        |
| 619,017   | 4/1961  | Canada.        |
| 739,408   | 7/1966  | Canada.        |
| 1,146,218 | 5/1957  | France.        |
| 977,105   | 12/1964 | Great Britain. |
| 999,482   | 7/1965  | Great Britain. |

RICHARD O. DEAN, Primary Examiner

U.S. CL. X.R.

75-53, 58, 59